



US006004629A

# United States Patent [19]

Madigan

[11] Patent Number: 6,004,629

[45] Date of Patent: Dec. 21, 1999

[54] **PROCESS FOR APPLYING A COATING TO SHEET METAL**[76] Inventor: **William Vincent Madigan**, 27 Washington Ave. P.O. Box 87, Bayville, N.Y. 11709[21] Appl. No.: **08/887,477**[22] Filed: **Jul. 2, 1997**[51] Int. Cl.<sup>6</sup> ..... **C08F 2/46**[52] U.S. Cl. ..... **427/496; 427/327; 427/385.5; 427/409; 427/435; 427/551; 427/560; 427/601**[58] **Field of Search** ..... **427/496, 551, 427/560, 601, 327, 385.5, 409, 435**[56] **References Cited**

## U.S. PATENT DOCUMENTS

4,410,560 10/1983 Kosterka ..... 427/44  
4,788,992 12/1988 Swainbank et al. ..... 134/64

## OTHER PUBLICATIONS

"UV/EB Curing Primer 1", RadTech International North America, Jan. 1995, pp. 1-3, 11, 12.

Molenar, New electron beam curing facility at TNO: perspectives for coil coating, European polymers, paint &amp; colour Journal, Mar. 1990, pp. 148.

Smit, et al, "Investigations on the Adhesion of EB cured coatings on Metal Substrates", TNO Centre for Coating Research, about 1992 No Month Avail.

"Electron Beam Basics", Energy Sciences Inc. trade literature, 1994, pp. 1-8 (No Month Avail).

Primary Examiner—Bernard Pianalto  
Attorney, Agent, or Firm—Harry L. Newman[57] **ABSTRACT**

A process for coating sheet metal is disclosed that comprises the steps of 1) cleaning the sheet metal to remove surface contaminants that may interfere with the coating adhering to the sheet metal; 2) pretreating the sheet metal to promote adhesion of the coating to the sheet metal; 3) applying an electron beam curable coating to the sheet metal that when curing is complete, adheres to the sheet metal; and, 4) exposing the coating on the sheet metal to an electron beam to cure the coating, the cleaning, pretreating and curing resulting in no emission of pollutants that need to be removed before the emission is released into the atmosphere.

**9 Claims, 3 Drawing Sheets**







## PROCESS FOR APPLYING A COATING TO SHEET METAL

### FIELD OF THE INVENTION

This invention is directed to the field of coating sheet metal and more particularly, to a process for coating sheet metal that does not result in the emission of pollutants that need to be removed before the emission is released into the atmosphere.

### BACKGROUND OF THE INVENTION

The traditional method of coating sheet metal is to apply a solvent or water-based coating to the sheet metal, and then move the sheet metal through an oven to cure the coating. The curing is accomplished by heating the sheet metal and the coating to a temperature at which the solvent or water in the coating is evaporated and at which the coating itself is not harmed. To obtain a uniform coating and for greatest efficiency and lowest cost, the curing is a continuous process in which 1) the oven needs to be maintained at a constant temperature, 2) the sheet metal needs to be continuous and 3) the sheet metal needs to be moved through the oven at a constant rate of speed. A typical rate is 200 to 400 feet per minute.

To meet the requirement that the sheet metal be continuous, two pay off coils of sheet metal and a welder/joiner need to be provided. The sheet metal is advanced from one of the pay off coils, and when the end of that coil is reached, it is welded to the beginning of the second pay off coil. Then, as sheet metal is advanced from the second coil, the exhausted first coil is replaced. In addition, after the coating on the sheet metal is cured, the sheet metal needs to be re-coiled. To accomplish this, a shear and two re-coil mechanisms need to be provided. The continuously moving sheet metal is wound on a first re-coil mechanism, and when the desired coil size is reached, the sheet metal is cut by the shear. The sheet metal is then wound on the second re-coil mechanism while the coil on the first re-coil mechanism is removed.

Both the welding/joining operation at the beginning of the process and the shearing operation at the end of the process require interruption of the movement of the sheet metal. Therefore, to satisfy the requirement that the sheet metal move through the oven at a constant rate of speed, it is necessary that a first excess length of sheet metal be provided after the welder/joiner. This excess length of sheet metal is fed into the process during the time that the welding/joining operation is taking place and no sheet metal is being advanced from one of the pay off coils. It is apparent that even at the modest rate of speed of 200 to 400 feet per minute, allowing for the worst case interruption requires that the excess length of sheet metal be substantial.

This excess length of sheet metal is provided by apparatus referred to as an accumulator. This accumulator is typically a tower within which the excess sheet metal is vertically looped back and forth on itself in serpentine fashion. The ends of the loops are wrapped around rollers that move toward one another to shorten the loops when excess length is being used to replace the sheet metal not being provided by a pay off coil. Once the welding/joining operation is completed, the rollers move away from one another as the desired excess length is restored in the accumulator.

A second accumulator needs to be provided before the shear and re-coil mechanisms. This is because the sheet metal is continuously moving out of the oven at the constant rate of speed. During the time when the winding of the sheet

metal is being transferred from one of the re-coil mechanisms to the other, the sheet metal needs to be accumulated. In the second accumulator, the length of the loops are increased when no re-coil mechanism is in operation and decreased when a re-coil mechanism is in operation. The oven used in the traditional method needs to be of considerable length in order to effect complete curing of the coating applied to the sheet metal. A length of 100 feet for sheet metal of 0.050 thickness moving at a rate of 200 to 400 feet per minute is appropriate. Of course, the length of the oven needs to be increased if the thickness of the sheet metal and/or the rate at which the sheet metal moves through the oven is increased.

Prior to the coating being applied to the sheet metal, the sheet metal needs to be cleaned to remove contaminants that may interfere with the coating adhering to the sheet metal and pretreated to promote adhesion of the coating to the sheet metal. In the traditional method, both the materials used in the cleaning of the sheet metal and the materials used in the pretreating of the sheet metal contain pollutants in the form of volatile organic compounds that are emitted during the cleaning and pretreating operations. These pollutants need to be removed before the emissions can be released to the atmosphere.

Similarly, the coating used in the traditional method contain volatile organic compounds that are emitted during the curing operation. Again, these pollutants need to be removed before the emissions can be released to the atmosphere. It is, therefore, necessary in the traditional method to have in place pollution control equipment that removes these pollutants from the emissions exhausted from the cleaning operation, the pretreating operation, and the curing operation.

It is seen from the above that the traditional method for coating sheet metal has many deficiencies. First, it requires large amounts of equipment and a building of substantial size to house the equipment. Thus, it requires a significant investment of capital. Second, without a substantial increase in capital investment, it is a relatively low speed process. Third, it only lends itself to long runs. A coating line needs to operate around the clock for days or weeks once coating of sheet metal with a coating of a particular color has begun. Fourth, because of this and the many pieces of equipment involved in this process, the cost of operation and maintenance is significant. Last, and most importantly, it requires the installation of pollution control equipment to prevent pollution of the atmosphere.

### SUMMARY OF THE INVENTION

The sheet metal coating process, in accordance with the present invention, provides very significant advantages over the traditional coating method.

The process, in accordance with the present invention, uses an electron beam curable coating rather than a heat curable coating. Consequently, the curing oven is eliminated along with the need to have a continuous length of sheet metal moving at a constant rate of speed. As a result, the second pay off mechanism, the two accumulator towers, and the second re-coil mechanism are all unnecessary. If individual sheets rather than a coil is being coated, then the welder/joiner and shear can also be eliminated. The equipment necessary to carry out the sheet metal coating process in accordance with the present invention is, therefore, far less costly than that required for the traditional method. In addition, because there is less equipment than in the traditional method, the cost of operating and maintaining the equipment is also reduced.

Another advantage of the coating process in accordance with the present invention is the rate of speed at which the sheet metal can be coated. Without increasing the cost of the equipment from that stated above, the sheet metal can be coated and cured at a rate of speed of 600 to 800 feet per minute. To provide this same rate with the traditional method would result in the equipment cost almost doubling.

Still another advantage of the coating process in accordance with the present invention is that it can accommodate not only long production runs, but also short ones. With the coating used in the traditional method, the coating cures even at ambient temperatures. The coating used in the present invention, on the other hand, only cures when it is exposed to an electron beam. Thus the system can be purged, the coating recovered, and the equipment that applies the coating to the sheet metal readily cleaned. The process in accordance with the present invention can, therefore, be used to do short custom runs. It can also be used to provide coated sheet metal in small batches on a just-in-time basis. This allows the purchaser to reduce their inventory and save money.

Most importantly, the coating process of the present invention is environmentally friendly in that it does not result in the emission of pollutants. The term "pollutant" as used in this patent is defined to mean anything characterized by the U.S. Environmental Protection Agency (EPA) as an air pollutant that exceeds limits established by the EPA. The cleaning of the sheet metal to remove contaminants, in accordance with one embodiment of this invention, is accomplished ultrasonically. This is a water-based, rather than solvent-based, technology, and biodegradable aqueous detergents are available as an additive to the water washing solution. Following the washing of the sheet metal, it is given a clean water rinse and then dried. This cleaning operation does not result in the emission of pollutants.

Second, the pretreating of the sheet metal to promote adhesion of the coating to the sheet metal, in accordance with one embodiment of this invention, is accomplished using a water-based pretreatment solution that does not emit pollutants.

Finally, coating the sheet metal is accomplished using electron beam technology rather than an oven which cures the coating by evaporating the liquid in the coating. During the electron beam processing, electrons in the coating liquid are redistributed and the coating is transformed into a solid through the process of polymerization and crosslinking. The transformation of the coating into a solid is virtually instantaneous and produces no emissions.

Thus, it is seen that the cleaning and pretreating of the sheet metal and the curing of the coating does not result in the emission of pollutants that need to be removed before the emission is released to the atmosphere.

#### BRIEF DESCRIPTION OF THE DRAWINGS

The sheet metal coating process in accordance with the present invention will be more fully described with reference to the following drawing figures of which:

FIG. 1 is a schematic drawing illustrating one application of the process of the present invention;

FIG. 2 is a schematic drawing illustrating ultrasonic apparatus; and

FIG. 3 is a schematic drawing illustrating electron beam curing apparatus.

#### DETAILED DESCRIPTION OF THE INVENTION

FIG. 1 illustrates the application of the process of the present invention to the coating of both sides of a coil of

sheet metal. Sheet metal 10 is advanced from a coil 100 mounted on pay off apparatus 110 and moved through a welder/joiner 150 via rollers 120. The welder/joiner 150 serves to join the tail end of an exhausted coil with the beginning end of a fresh coil. This avoids having to manually thread the beginning end of the fresh coil through the system. Such equipment is available from Newcor in Bay City, Mich. From the welder/joiner the sheet metal 10 moves via rollers 160 into cleaning apparatus 200. The function of the cleaning apparatus 200 is to remove surface contaminants that may interfere with the coating, which is subsequently applied to the sheet metal 10, from adhering to the sheet metal. These contaminants include dirt, oil and grease. This cleaning operation is accomplished in three steps: first, the surface of the sheet metal 10 is cleaned; second, the surface is rinsed; and third, the surface is dried in preparation for the next step in the process.

Referring to FIG. 2, one embodiment of cleaning apparatus 200 for performing the cleaning operation without resulting in the emission of pollutants is shown. The cleaning apparatus 200 comprises an ultrasonic cleaning section 220, rinsing section 240, and a drying section 260. The cleaning section 220 includes multiple pairs of opposing ultrasonic transducers 222 and 224. The ultrasonic transducers 222 and 224 are closely spaced and operate at different frequencies. Both the sheet metal 10 and a washing solution 225 move through the space between the opposing faces of each pair of ultrasonic transducers 222 and 224. The operation of the ultrasonic transducers 222 and 224 in combination with the washing solution 225 provides ultrasonic cleaning of both sides of the sheet metal 10. The washing solution 225 can be just water or a mild emulsifying soap or biodegradable aqueous detergent can be added to the water to enhance the cleaning action of the ultrasonic transducers 222 and 224. The sheet metal 10 and washing solution 225 advantageously move in opposite directions, the washing solution carrying away the contaminants and flowing into a collector chamber from which it is drained, filtered and recirculated.

The sheet metal 10 moves from the cleaning section 220 into the rinsing section 240. In this section multiple pairs of opposed rinse water nozzles 242 spray both surfaces of the sheet metal 10, the nozzles comprising each pair being on opposite sides of the sheet metal. As the sheet metal 10 moves between successive pairs of rinse nozzles 242, any of the washing solution 225 remaining on the sheet metal is removed. The rinse water applied by the initial pairs of nozzles 242 may be recirculated while the rinse water applied by the final pairs of nozzles may be fresh water.

In the final step of the cleaning process, the sheet metal 10 is moved into the drying section 260. In the section multiple pairs of opposed air knives 262 are used to blow the rinse water off of both surfaces of the sheet metal 10, the air knives comprising each pair being on opposite sides of the sheet metal. Compressed air, which is heated as a result of its compression, is advantageously provided to the air knives 262. As a result, the sheet metal 10 leaving the drying section 260 is essentially dry. A more detailed description of ultrasonic strip cleaning apparatus is provided in U.S. Pat. No. 4,788,992.

Referring again to FIG. 1, the sheet metal 10 leaving the cleaning apparatus 200 moves on to pretreatment solution application apparatus 300. The pretreatment solution application apparatus 300 includes two pretreatment solution reservoirs 310. Each pretreatment solution reservoirs 310 is associated with a group of interacting rollers 320 for picking up the pretreatment solution from the reservoir and applying

it to one side of the sheet metal **10**. The rollers **320** respectively associated with the pretreatment solution reservoirs **310** are on opposite sides of the sheet metal **10**, and therefore, the pretreatment solution is applied to both sides of the sheet metal as it moves through the pretreatment solution application apparatus **300**.

The pretreatment solution applied to the sheet metal **10** is then dried by moving the sheet metal through an oven **400**, that uses infrared heating elements, such as one manufactured by BGK, an Illinois Tool Works Company in Minneapolis, Minn. This pretreatment of the sheet metal **10** serves to promote adhesion of the subsequently applied coating to the sheet metal surfaces. In accordance with the present invention, the pretreatment solution that is applied to the sheet metal **10** comprises a material that does not emit pollutants when it is applied and dried. An example of such a product is Organokrome 2000 Pretreat available from the Coatings and Resins Group of PPG Industries Inc.

After both sides of the sheet metal **10** have been pretreated, the sheet metal moves to coating apparatus **500**. The coating apparatus **500** includes a coating liquid reservoir **510** and a group of interacting rollers **520** that pick up an electron beam curable coating liquid from the reservoir and apply it to the bottom surface of the sheet metal **10**. An example of such a coating that has been found to achieve a good bond to the sheet metal **10** once curing is completed is Durethane. This product is available from the Coatings and Resins Group of PPG Industries Inc. After the application of the coating, the sheet metal **10** moves to electron beam curing apparatus **600**.

Referring now to FIG. 3, the electron beam curing apparatus **600** comprises a high voltage power supply **610** that provides power to an electron gun assembly **620**, positioned within a vacuum chamber **630** having a foil window **632** on one side. The foil window **632** is mounted on the underside of a center portion **642** of a conduit **640**. The center portion **642** extends at an angle to an entrance portion **644** and an exit portion **645** at each end of the center portion, the entrance and exit portions extending generally parallel to one another. Rollers **646** and **647** respectively positioned within the entrance portion **644** and exit portion **645** serve to guide the movement of the sheet metal **10** through the conduit **640**.

The electron gun assembly **620** includes tungsten filaments (not shown) and when high voltage is applied to the filaments, a cloud of electrons is generated. Electrons are drawn from the cloud to areas of lesser voltage of the gun assembly, and the electrons accelerate to extremely high speeds. The electrons exit the vacuum chamber through and generally perpendicular to the foil window **632** and penetrate the coating of the underside of the sheet metal **10** moving through the conduit **640**. As a result, the coating is transformed into a solid through the process of polymerization and crosslinking. Electron beam polymerization is the process in which several individual groups of molecules combine together to form one large group called a polymer. Electron beam crosslinking is the process by which an interconnected network of chemical bonds or links develop between polymer chains to form a stronger molecular structure. Many coatings require a low oxygen environment during electron beam processing to be able to convert from a liquid to a solid. Therefore, nitrogen gas is pumped into the conduit **640** through jets (not shown) to displace the oxygen that would prevent complete curing. Finally, the shape of the conduit **640** serves to prevent electrons from escaping through the entrance and exit ports **644** and **645**. Electron beam curing apparatus of the type described is manufactured

by RPC Industries in Hayward, Calif. and Energy Sciences Inc. in Wilmington, Mass.

Referring again to FIG. 1, the sheet metal **10** leaving the electron beam curing apparatus **600** moves to coating apparatus **700**. The coating apparatus **700** includes a coating liquid reservoir **710** and a group of interacting rollers **720** that pick up an electron beam curable coating liquid from the reservoir and apply it to the top surface of the sheet metal **10**. The sheet metal **10** then moves to electron beam curing apparatus **800**.

The electron beam curing apparatus **800** is the same as electron beam curing apparatus **600** previously described except that the orientation is changed to apply the electron beam to the top surface of the sheet metal **10** to cure the coating applied by the coating apparatus **700**.

The final step of the process is to rewind the sheet metal **10** into a coil. This is accomplished by the sheet metal re-coil apparatus **900**. A shear **950** is advantageously located before the re-coil apparatus **900** to cut the sheet metal **10** when the coil on the re-coil apparatus has reached the appropriate size. Such a shear is available from Hallden America in Thomaston, Conn.

While the preferred embodiment of this invention has been described in the Detailed Description, the scope of the invention is defined in the following claims.

What is claimed is:

1. A process for coating a continuous moving length of sheet metal comprising the steps of:

Cleaning the moving length of sheet metal with a water based solution to remove surface contaminants that may interfere with the coating adhering to the sheet metal;

Applying a water based pretreatment solution to the moving length of sheet metal to promote adhesion of the coating to the surface of the sheet metal;

Applying an electron beam curable coating to the moving length of sheet metal; and

Exposing the moving length of sheet metal to an electron beam to cure the coating.

2. The process as in claim 1 wherein the step of cleaning the moving length of sheet metal comprises the substeps of:

a) Ultrasonically cleaning the surface of the moving length of sheet metal in a washing solution to remove surface contaminants that may interfere with the coating adhering to the sheet metal, the washing solution carrying away the contaminants removed from the sheet metal by the ultrasonic cleaning;

b) Rinsing the surface of the moving length of sheet metal to remove the washing solution; and

c) Drying the surface of the moving length of sheet metal to remove the rinsing solution.

3. The process as in claim 2 wherein the step of pretreating the moving length of sheet metal comprises the substeps of

a) Applying a water based pretreatment solution to the surface of the sheet metal; and

b) Drying the pretreatment solution to provide a dry pretreated surface for the application of the electron beam curable coating.

4. A process for coating a continuous moving length of sheet metal comprising the steps of:

Cleaning the moving length of sheet metal to remove surface contaminants that may interfere with the coating adhering to the sheet metal;

Pretreating the moving length of sheet metal to promote adhesion of the coating to the surface of the sheet metal;

Applying an electron beam curable coating to the moving length of sheet metal that adheres to the sheet metal when curing is complete; and

Exposing the moving length of sheet metal to an electron beam to cure the coating;

The cleaning, pretreating, and curing resulting in no emission of pollutants that need to be removed before the emission is released into the atmosphere.

5. The process as in claim 4 wherein the step of cleaning the moving length of sheet metal comprises the substeps of:

a) Ultrasonically cleaning the moving length of sheet metal in a washing solution for carrying away the contaminants removed from the sheet metal by the ultrasonic cleaning;

b) Rinsing the moving length of sheet metal to remove the washing solution; and

c) Drying the moving length of sheet metal to remove the rinsing solution.

6. The process as in claim 5 wherein the step of pretreating the moving length of sheet metal comprises the substeps of:

a) Applying a water-based pretreatment solution to the surface of the sheet metal; and

b) Drying the pretreatment solution to provide a dry pretreated surface for the application of the electron beam curable coating.

7. A process for coating a sheet metal coil comprising the steps of:

Advancing the sheet metal from the coil to provide a continuous and moving length of sheet metal;

Ultrasonically cleaning the surface of the moving length of sheet metal in a washing solution to remove surface contaminants that may interfere with the coating adhering to the sheet metal, the washing solution carrying away the contaminants removed from the sheet metal by the ultrasonic cleaning;

Rinsing the surface of the moving length of sheet metal to remove the washing solution;

Drying the surface of the moving length of sheet metal to remove the rinsing solution;

40 Applying a water-based pretreatment solution to the surface of the moving length of sheet metal to promote adhesion of the coating to the surface of the sheet metal;

10

15

20

25

30

35

40

Drying the pretreatment solution on the moving length of the sheet metal to provide a dry pretreated surface for the application of the coating;

Applying an electron beam curable coating to the moving length of the sheet metal which when curing is complete adheres to the sheet metal; and

Exposing the moving length of sheet metal to an electron beam to cure the coating;

The cleaning, pretreating, and curing resulting in no emission of pollutants that need to be removed before the emission is released into the atmosphere.

8. A process for coating a continuous moving length of sheet metal comprising the steps of:

Ultrasonically cleaning the moving length of sheet metal in a water based washing solution to remove surface contaminants that may interfere with the coating adhering to the sheet metal;

Applying a water based pretreatment solution to the moving length of sheet metal to promote adhesion of the coating to the surface of the sheet metal;

Applying an electron beam curable coating to the moving length of sheet metal; and

Exposing the moving length of sheet metal to an electron beam to cure the coating.

9. A process for coating a continuous moving length of sheet metal comprising the steps of:

Cleaning the moving length of sheet metal using a non-solvent based technology to remove surface contaminants that may interfere with the coating adhering to the sheet metal;

Applying a water based pretreatment solution to the moving length of sheet metal to promote adhesion of the coating to the surface of the sheet metal;

Applying an electron beam curable coating to the moving length of sheet metal; and

Exposing the moving length of sheet metal to an electron beam to cure the coating.

\* \* \* \* \*